

## UNITED STATES PATENT OFFICE

ARTHUR L. KENNEDY, OF KEENE, NEW HAMPSHIRE, ASSIGNOR TO PLASTIC, INC., A CORPORATION OF NEW HAMPSHIRE

## MINERAL FIBER PAPER AND PROCESS OF MAKING THE SAME

No Drawing.

Application filed June 22, 1927. Serial No. 200,773.

My invention relates particularly to a paper containing a mineral fiber, such, for example, as asbestos or mineral wool, and the process of making the same, and which has 5 many advantages over previous papers made from mineral fibers.

The object of my invention is to provide a paper containing a mineral fiber, as, for example, asbestos or mineral wool, but which 10 has very superior characteristics over previous asbestos papers and similar products, and the object is, also, to provide an advantageous process for the making of the same.

Previously, in the manufacture of asbestos paper it has been found necessary to include therein a large amount of vegetable fiber, the minimum amount of this fiber required being usually 40%, in order to avoid continual breakage in the web, so as to produce 15 the desired flow of the wet pulp, to prevent the web sticking to the rolls, and, furthermore, to avoid producing holes and pock marks in the finished papers. Also, in using asbestos papers made in accordance with previous 20 processes, as, for example, in the winding of electric wires and cables, the manufacturer found it necessary to count upon a very large percentage of loss due to breakage of the paper in the winding operations.

The paper made in accordance with my invention does not require the presence of any vegetable fiber whatever, and, furthermore, can be made with a very much larger percentage of asbestos or other mineral fiber. Nevertheless, a paper made in accordance with my invention has a greater strength, takes a much smoother finish, and is very much more flexible than previous asbestos papers. Furthermore, by reason of the increased strength the large percentage of breakages, as in the use of previous asbestos papers, is avoided, thus materially decreasing the cost of manufacture and the cost of working the paper into manufactured products.

The paper made in accordance with my invention has a wide variety of uses and is especially applicable to the winding of electric wires and cables, not only by reason of the small percentage of the breakage, but, also, because of the very high dielectric of the pa-

per. In fact, it is adapted to be used to great advantage wherever electric resistance is desired, and has, of course, many other uses.

While my invention is capable of embodiment in many different forms, and of being carried out in many different ways, for the purpose of illustration I shall describe only certain forms of the same hereinafter.

The paper made in accordance with my invention contains kelp, that is to say, sea-weed, as, for example, a marine plant known as "laminaria". Other forms of sea-weed may be used, if desired, however.

As one example of my invention, 1000 lbs. of kelp while wet and preferably with the stems removed, which comprises approximately 100 lbs. of solids by dry weight, are mixed with 15 lbs. of soda ash, that is to say, sodium carbonate, or any other form of alkali. These are ground up in any desired kind of apparatus for comminuting the same, such, for instance, as a meat-chopper. To the mass thus obtained I add a 10% solution of sulphuric acid in water in just sufficient quantity to neutralize the alkali. This produces a coagulated precipitate which is then washed in three wash waters to eliminate the natural mineral salts of the kelp, such as sodium, potassium, calcium, iodine, bromine, iron, and sulphur compounds. The purpose of this stop is to prevent the subsequent crystallization of these salts in the paper, which would interfere with the dielectric of the latter. The water is then removed from the coagulated precipitant, either in a press to form press-cakes, or in a rotary centrifuge, thus obtaining a kelp product ready for admixture with the mineral fibers. The mineral fibers may be asbestos, mineral wool, or any other desired kind of mineral fiber.

15 lbs. of the kelp product are then mixed with 100 lbs. of asbestos, using, preferably, asbestos fibers, having a length of  $1\frac{1}{4}$ " or more. If desired, however, a fiber shorter than  $1\frac{1}{4}$ " length may be used, although the  $1\frac{1}{4}$ " length fibers are preferred.  $2\frac{1}{4}$  lbs. of sodium carbonate are then added, as well as 75 gals. of water, and the kelp mixture is then subjected to the action of a beater to thoroughly mix the same. When they are

completely mixed there are added to the mass 3 lbs. of calcium chloride or calcium acetate, or, in fact, any other soluble metallic salt that will produce an insoluble compound with 5 the alginic acid of the kelp. The algulose which is also present may or may not combine in part or wholly with the said salt. The pulp thus formed is then run into an ordinary paper making machine, such, for example, as is used in the production of news- 10 paper print or book papers, and which, in general, comprises a web forming part, a drying part, and a calendering part. There- 15 after, the web formed from the pulp as above described, is put through a super-calender, that is to say, a calender having rolls heated to a temperature of 115° C., so as to give added strength and gloss to the product. Asbestos papers made in accordance with 20 previous processes could not be subjected to the super-calendering step without becoming more brittle and liable to crack so as to tend to make the larger asbestos fibers fall out and thus form perforations in the paper. On the 25 contrary, in the product made in accordance with my invention, the use of the super-calendering step makes the product softer than before the super-calendering treatment.

While I have described my invention above 30 in detail I wish it to be understood that many changes may be made therein without departing from the spirit of the same.

I claim:

1. The process which comprises forming 35 a paper web from a pulp containing a mineral fiber and a kelp product precipitated therein from alginic acid by a mineral salt adapted to form an insoluble compound therewith, the alginic acid having been produced by grinding the kelp with an alkali, neutralizing with an acid, washing, and then removing the water therefrom.

2. The process which comprises forming a paper web from a pulp containing asbestos 45 and a kelp product precipitated therein from alginic acid by a mineral salt adapted to form an insoluble compound therewith, the alginic acid having been produced by grinding the kelp with an alkali, neutralizing with an acid, washing, and then removing the water therefrom.

3. The process which comprises forming 55 a paper web from a pulp containing a mineral fiber and a kelp product precipitated therein from alginic acid by a mineral salt adapted to form an insoluble compound therewith, the alginic acid having been produced by grinding the kelp with an alkali, neutralizing with an acid, washing, and then removing the water therefrom so as to form 60 press-cakes.

4. The process which comprises forming a paper web from a pulp containing asbestos and a kelp product precipitated therein from 65 alginic acid by a mineral salt adapted to form

an insoluble compound therewith, the alginic acid having been produced by grinding the kelp with an alkali, neutralizing with an acid, washing, and then removing the water therefrom so as to form press-cakes. 70

5. The process which comprises forming a kelp product by grinding the kelp with an alkali, neutralizing the alkali with an acid, washing, and then removing the water therefrom. 75

6. The process which comprises forming a kelp product by grinding the kelp with an alkali, neutralizing the alkali with an acid, washing, and then removing the water therefrom in a press to form press-cakes. 80

7. The process of making paper which comprises treating kelp with an alkali to solubilize the alginic acid and algulose, coagulating with a mineral acid, washing to eliminate natural mineral salts, incorporating fiber pulp with the coagulated material and forming paper therefrom. 85

8. A mineral fiber paper consisting essentially of mineral fiber pulp and a kelp product formed from kelp, including its alginic acid and algulose which has been solubilized with an alkali and rendered insoluble with a precipitant. 90

9. An asbestos paper consisting essentially of asbestos fiber and a kelp product formed from kelp, including its alginic acid and algulose which has been solubilized with an alkali and rendered insoluble with a precipitant. 95

10. A mineral fiber paper consisting essentially of mineral fiber pulp and a kelp product formed from kelp including its alginic acid and algulose which has been solubilized and then rendered insoluble by the addition of a mineral acid. 100 105

In testimony that I claim the foregoing, I have hereunto set my hand this 17th day of June, 1927.

ARTHUR L. KENNEDY.

110

115

120

125

130